# EUROPEAN PATENT APPLICATION

(11) **EP 0 995 709 A2**
(43) Date of publication of application: **26.04.2000**
(21) Application number: 99101075.2
(22) Date of filing: 25.01.1999
(51) Int. Cl.: B65H 27/00, B65H 3/06

(54) **Sheet feeder for office machines and process for its manufacture**

(30) Priority: 21.10.1998 IT TO980895
(71) Applicant: S.I.V.E. S.p.A., 10073 Cirie (Torino) (IT)
(72) Inventor: Giordano, Nicola, 10073 Ciriè (Torino) (IT)
(74) Representative: Aprà, Mario

(57) **Abstract**

In a sheet feeder for office machines, in which the advance in the desired direction of each of a plurality of sheets stacked in a magazine is caused by at least one rotating feed shaft and/or feed members integral with the shaft, according to the invention the friction surface of the feed shaft, or of the feed members integral with it, consists of a surface coating of rubberized enamel, applied as a paint and incorporating a particulate of a rubber resin, in such a way that the said surface coating imparts to the friction surface of the feed shaft, or of the feed members integral with it, a surface softness which increases with an increase in the thickness of the coating layer and a surface friction which makes it pleasant to touch ("soft touch") and suitable for feeding sheets, particularly sheets of paper.

## Description

The present invention relates to a sheet feeder for office machines. The invention also relates to a process for the manufacture of this feeder. A known sheet feeder of the specified type generally comprises a rotating feed shaft which may be provided with integral friction members which, by rotating in contact with the surface of a sheet, cause it to advance in the desired direction. These friction members consist, for example, of feed rollers keyed coaxially to the feed shaft.

Additionally, in photocopying and facsimile machines and in all types of printers (impact, laser and ink-jet), and in similar known office machines, the paper sheet is fed by means of a feed shaft, as indicated above, opposed to rollers or blocks of "soft" material. This arrangement makes it possible to divide a number of sheets stacked in a magazine into single sheets and to advance them in sequence, picking them off one by one in the desired direction. However, for this condition to be met, the coefficient of friction (Ka) of the various members must conform to the following relation: in which:
Ka R1 is the coefficient of friction between the feed member (for example, a feed roller) and the sheet to be fed;
Ka R2 is the coefficient of friction between the member opposed to the feed member and the sheet to be fed;
Ka F is the coefficient of friction between the stacked sheets.

This relation must also be kept as constant as possible during the whole required lifetime of the feed member, corresponding to approximately one hundred thousand sheets.

Evidently, the choice of material from which the feed shaft and/or the feed roller is made is a determining factor for the satisfactory operation of the system.

The feed members used at the present time are:
metal rollers whose friction surface is roughened by subsequent machining;
rubber rollers provided with suitable additives and machined to provide a surface roughness suitable for feeding.

The use of these materials causes certain problems which are not easily resolved.

In the first case, in addition to the rather high manufacturing costs, the jamming of the sheets of paper may cause their deterioration as a result of abrasion.

In the second case, the dust produced by the abrasion of the sheets during their advance is deposited on the rollers, thus reducing the value of Ka R1.

The principal object of the present invention is, therefore, to provide a sheet feeder for office machines which does not abrade the paper and which, after a normal initial loss, has a coefficient of friction which is stabilized at a virtually constant level in time, throughout its service life.

Another object is to provide a sheet feeder as specified which is structurally simplified and requires a smaller technical and economic outlay for its manufacture.

It is also an object of the invention to provide a process for manufacturing a sheet feeder for office machines which can be simply and economically implemented.

In accordance with these objects, the present invention provides a sheet feeder for office machines, whose essential characteristic forms the subject of the principal claim.

The process according to the present invention forms the subject of Claim 2.

Further advantageous characteristics are described in the subsidiary claims.

The claims are to be understood as being stated in full herein.

According to the present invention, the friction surface of the feed shaft, or of the feed members integral with it, consists of a surface coating of rubberized enamel applied as a paint and incorporating a particulate of rubber resin.

This surface coating imparts to the friction surface of the feed shaft, or of the feed members integral with it, a surface softness which increases with an increase in the thickness of the surface layer and a surface friction which makes it pleasant to touch ("soft touch") and suitable for feeding, particularly for feeding sheets of paper.

The principal advantages of the sheet feeder for office machines according to the invention are:
- greater stability; minimizing of the "buffer" effect;
- greater dimensional accuracy;
- a virtual absence of wear;
- high tractive force;
- a coefficient of friction which is constant over time.

All these properties impart to the sheet feeder according to the invention characteristics which are manifested, in the final analysis, in a significant reduction of costs. The process according to the invention for the manufacture of the aforesaid sheet feeder for office machines essentially comprises the following stages:
* surface preparation of the part;
* painting the part with rubberized enamel;
* baking.

These stages are advantageously preceded by the following stage:
* determination of the thicknesses (design of the part, namely the feed shaft and/or feed members integral with it).

Preferably, the parts to be treated by the process according to the invention are made from iron, nickel-plated iron, or ABS (acrylonitrile-butadiene-styrene), and are suitably prepared to ensure the adhesion of the surface coating of rubberized enamel and corrosion-resistance.

Specifically, the aforesaid stages comprise the execution of the following processes.

### 1. Preliminary determination of the thicknesses

This operation provides a high precision of the final tolerances of the part. It is necessary to design the part and the required tolerances with allowance for the thickness of rubberized enamel which is to be applied. The minimum tolerance required in the unfinished part is ± 20 µm (on the diameter), to give a final minimum tolerance of ± 50 µm.

### 2. Surface preparation

Iron parts require the preliminary application of a corrosion-proofing primer, which ensures good adhesion, on which the final rubberized enamel is to be applied. Black cataphoresis is the best preliminary treatment, with a deposition thickness of 12-15 µm.

Rubberized enamel does not adhere well to nickel-plated iron. Sanding with abrasive paper is required on the areas to be painted with rubberized enamel.

For parts made from synthetic resins, particularly ABS (acrylonitrile-butadiene-styrene), sanding to roughen their surfaces is required.

### 3. Painting with rubberized enamel.

Rubberized enamel is a paint which incorporates a particulate of rubber resin. This imparts to the surface of the parts coated with the rubberized enamel a surface softness, which increases with an increase in the thickness of paint, and a surface friction which makes it pleasant to touch ("soft touch") and suitable for feeding sheets of paper in particular.

### 4. Baking

The baking stage polymerizes the rubberized enamel and increases its adhesion to the coated part.

Naturally, many modifications may be made.

The surface coating may contain additives of friction material (for example, quartz powder, aluminium oxide, expanded silica, etc.) for surface roughening. For the formation of the said layer, at least one rubberized enamel is mixed with a powdered or granular additive, and is then applied by mechanical means to the surface of the part to be coated.

## Claims

1. Sheet feeder for office machines, in which the advance in the desired direction of each of a plurality of sheets stacked in a magazine is caused by at least one rotating feed shaft and/or feed members integral with the shaft, characterized in that the friction surface of the feed shaft, or of the feed members integral with it, consists of a surface coating of rubberized enamel, applied as a paint and incorporating a particulate of a rubber resin, in such a way that the said surface coating imparts to the friction surface of the feed shaft, or of the feed members integral with it, a surface softness which increases with an increase in the thickness of the coating layer and a surface friction which makes it pleasant to touch ("soft touch") and suitable for feeding sheets, particularly sheets of paper.

2. Feeder according to Claim 1, characterized in that the said surface coating contains additives of friction material (for example, quartz powder, aluminium oxide, expanded silica, or similar) for surface roughening.

3. Process of manufacturing a sheet feeder for office machines according to Claim 1 or 2, from an unfinished part forming a feed shaft and/or feed members which are integral or to be made integral with the shaft, characterized in that it comprises in succession the following operating stages:
surface preparation of the part;
surface coating of the part by painting with rubberized enamel;
baking of the surface coating of the part,
the part to be treated being advantageously made from iron, nickel-plated iron or ABS (acrylonitrile-butadiene-styrene), suitably prepared to ensure the adhesion of the surface coating of rubberized enamel and corrosion resistance.

4. Process according to Claim 3, characterized in that the said stage of surface preparation of the part comprises:
- for iron parts, the preliminary application of a corrosion-proofing primer, which ensures good adhesion and on which the final rubberized enamel is to be applied (black cataphoresis being the preferable preliminary treatment, with a deposition thickness of 12-15 µm);
- for nickel-plated iron, sanding with abrasive paper on the areas to be painted with rubberized enamel, and
- for synthetic resin parts, particularly ABS, sanding to impart roughness to their surfaces.

5. Process according to Claim 3, characterized in that the said painting with rubberized enamel forms on the part a layer of coating having a surface softness which increases with the thickness of the layer of paint and a surface friction which makes it pleasant to touch ("soft touch") and suitable for feeding sheets, particularly sheets of paper.

6. Process according to Claim 3, characterized in that in the baking stage the layer of rubberized enamel is polymerized and its adhesion to the coated part is increased.

7. Process according to Claim 3, characterized in that a preliminary stage of determining the thicknesses of the part is carried out, in which the part and the required tolerances are designed, with allowance for the thickness of the layer of rubberized enamel to be applied to the part.

8. Process according to Claim 3, characterized in that, for the formation of the surface coating of the part, at least one rubberized enamel is mixed with at least one powdered or granular additive, and subsequently applied by mechanical means to the surface of the part.
